



US010991491B2

(12) **United States Patent**  
**Horiuchi et al.**

(10) **Patent No.:** **US 10,991,491 B2**  
(45) **Date of Patent:** **\*Apr. 27, 2021**

(54) **PERMANENT MAGNET, AND MOTOR AND POWER GENERATOR USING THE SAME**

(71) **Applicant:** **KABUSHIKI KAISHA TOSHIBA**,  
Tokyo (JP)

(72) **Inventors:** **Yosuke Horiuchi**, Tokyo (JP); **Shinya Sakurada**, Tokyo (JP); **Tsuyoshi Kobayashi**, Kanagawa-ken (JP); **Keiko Okamoto**, Kanagawa-ken (JP); **Masaya Hagiwara**, Kanagawa-ken (JP)

(73) **Assignee:** **KABUSHIKI KAISHA TOSHIBA**,  
Tokyo (JP)

(\*) **Notice:** Subject to any disclaimer, the term of this patent is extended or adjusted under 35 U.S.C. 154(b) by 0 days.

This patent is subject to a terminal disclaimer.

(21) **Appl. No.:** **13/744,524**

(22) **Filed:** **Jan. 18, 2013**

(65) **Prior Publication Data**

US 2013/0241681 A1 Sep. 19, 2013

(30) **Foreign Application Priority Data**

Mar. 15, 2012 (JP) ..... JP2012-058866

(51) **Int. Cl.**

**H01F 1/01** (2006.01)

**H01F 1/055** (2006.01)

**C22C 19/00** (2006.01)

(52) **U.S. Cl.**

CPC ..... **H01F 1/015** (2013.01); **C22C 19/00** (2013.01); **H01F 1/0557** (2013.01)

(58) **Field of Classification Search**

CPC ..... H01F 1/0577; H01F 7/02; H01F 10/126  
See application file for complete search history.

(56) **References Cited**

**U.S. PATENT DOCUMENTS**

4,746,378 A 5/1988 Wysiekierski et al.  
5,781,843 A \* 7/1998 Anderson et al. ..... 419/29  
(Continued)

**FOREIGN PATENT DOCUMENTS**

JP 59023803 A \* 2/1984 ..... C22C 1/0441  
JP 59-118827 7/1984  
(Continued)

**OTHER PUBLICATIONS**

English Machine Translation of JP H06-212327.\*  
(Continued)

*Primary Examiner* — Xiaowei Su

(74) *Attorney, Agent, or Firm* — Amin, Turocy & Watson, LLP

(57) **ABSTRACT**

In one embodiment, a permanent magnet includes a composition expressed by  $R_pFe_qM_rCu_sCo_{100-p-q-r-s}$  ( $R$  is a rare-earth element,  $M$  is at least one element selected from Zr, Ti, and Hf,  $10 \leq p \leq 13.5$  at %,  $28 \leq q \leq 40$  at %,  $0.88 \leq r \leq 7.2$  at %, and  $3.5 \leq s \leq 13.5$  at %), and a metallic structure including a cell phase having a  $Th_2Zn_{17}$  crystal phase, and a cell wall phase. A Fe concentration ( $C1$ ) in the cell phase is in a range from 28 at % to 45 at %, and a difference ( $C1-C2$ ) between the Fe concentration ( $C1$ ) in the cell phase and a Fe concentration ( $C2$ ) in the cell wall phase is larger than 10 at %.

**10 Claims, 2 Drawing Sheets**



(56)

**References Cited**

## U.S. PATENT DOCUMENTS

|                  |         |                      |
|------------------|---------|----------------------|
| 8,568,539 B2     | 10/2013 | Horiuchi et al.      |
| 2002/0054825 A1* | 5/2002  | Sukaki .....         |
|                  |         | C22C 1/0441          |
|                  |         | 420/83               |
| 2012/0146444 A1* | 6/2012  | Horiuchi et al. .... |
| 2013/0076184 A1* | 3/2013  | Horiuchi et al. .... |
| 2013/0241333 A1  | 9/2013  | Horiuchi et al.      |
| 2013/0241682 A1* | 9/2013  | Horiuchi et al. .... |
|                  |         | 335/302              |

## FOREIGN PATENT DOCUMENTS

|                 |         |
|-----------------|---------|
| JP 63-149362    | 6/1988  |
| JP 06-212327    | 8/1994  |
| JP 07138672 A * | 5/1995  |
| JP 09-111383    | 4/1997  |
| JP 2011-216716  | 10/2011 |
| WO 2011016089   | 2/2011  |
| WO 2011121647   | 10/2011 |

## OTHER PUBLICATIONS

Huang et al. J of Applied Physics, 1994, vol. 75, p. 6280-6282.\*  
 TEM-EDX, <https://www.tcd.ie/Physics/ultramicroscopy/teaching/PY5019/notes/Nanoanalysis.pdf>, 2015.\*

Machine translation of JP07-138672A, May 1995.\*  
 Machine translation of JP59-023803A, Feb. 1984.\*  
 Translation of JP59-023803A, Feb. 1984.\*

Liu et al. (IEEE Transactions on Magnetics, 1989, vol. 25, No. 5, p. 3785-3787) (Year: 1989).\*

Japanese Office Action for Japanese Patent Application No. 2012-058866 dated Jan. 28, 2014.

Chinese Office Action for Chinese Patent Application No. 201310037671.0 dated Jan. 22, 2015.

Japanese Office Action for Japanese Application No. 2014-146194 dated Jun. 2, 2014.

Japanese Office Action for Japanese Application No. 2014-146195 dated Jun. 2, 2015.

Third Office Action for Chinese Patent Application No. 201310037671.0 dated Mar. 2, 2016, 9 pages.

Office Action of Notification of Reasons for Rejection for Japanese Patent Application No. 2014-146194 dated Jun. 2, 2015, 7 pages.

Office Action of Notification of Reasons for Rejection for Japanese Patent Application No. 2014-146195 dated Jun. 2, 2015, 7 pages

Ray, et al. "Recent Progress in 2:17-Type Permanent Magnets", Journal of Materials Engineering and Performance, vol. 1, No. 2, 1992, pp. 183-191, ISSN: 105-9495.

"Samarium Cobalt Permanent Magnets", Arnold the magnetic products group of SPS Technologies, Arnold\_SMCO\_Katalog, 2003, pp. 1-14.

\* cited by examiner

FIG. 1



FIG. 2



FIG. 3



## 1

## PERMANENT MAGNET, AND MOTOR AND POWER GENERATOR USING THE SAME

## CROSS-REFERENCE TO RELATED APPLICATION

This application is based upon and claims the benefit of priority from Japanese Patent Application No. 2012-058866, filed on Mar. 15, 2012; the entire contents of which are incorporated herein by reference.

## FIELD

Embodiments disclosed herein generally relate to a permanent magnet, and a motor and a power generator using the same.

## BACKGROUND

As a high-performance permanent magnet, there have been known rare-earth magnets such as a Sm—Co based magnet and a Nd—Fe—B based magnet. When a permanent magnet is used for a motor in a hybrid electric vehicle (HEV) or an electric vehicle (EV), the permanent magnet is required to have heat resistance. In a motor for HEV or EV, a permanent magnet whose heat resistance is enhanced by Dy substituting for part of Nd in the Nd—Fe—B based magnet is used. Since Dy is one of rare elements, there is a demand for a permanent magnet not using Dy. As a motor and a power generator with high efficiency, there have been known a variable magnetic flux motor and a variable magnetic flux power generator using a variable magnet and a stationary magnet. In order to improve performance and efficiency of the variable magnetic flux motor and the variable magnetic flux power generator, there is a demand for improvement in a coercive force and magnetic flux density of the variable magnet and the stationary magnet.

It is known that, because the Sm—Co-based magnet has a high Curie temperature, it exhibits excellent heat resistance without using Dy and is capable of realizing a good motor characteristic and so on at high temperatures. A  $\text{Sm}_2\text{Co}_{17}$  type magnet among the Sm—Co based magnets is usable as a variable magnet owing to its coercive force exhibiting mechanism and so on. Improvement in coercive force and magnetic flux density is also required of the Sm—Co-based magnet. In order to increase magnetic flux density of the Sm—Co based magnet, it is effective to increase Fe concentration, but the coercive force tends to decrease in a composition range where the Fe concentration is high. Under such circumstances, there is a demand for a technique for making a Sm—Co based magnet having a high Fe concentration exhibit a high coercive force.

## BRIEF DESCRIPTION OF THE DRAWINGS

FIG. 1 is a view showing a permanent magnet motor of an embodiment.

FIG. 2 is a view showing a variable magnetic flux motor of an embodiment.

FIG. 3 is a view showing a power generator of an embodiment.

## DETAILED DESCRIPTION

According to one embodiment, there is provided a permanent magnet including: a composition expressed by a composition formula:

## 2



where R is at least one element selected from rare-earth elements, M is at least one element selected from Zr, Ti, and Hf, p is a number satisfying  $10 \leq p \leq 13.5$  at %, q is a number satisfying  $28 \leq q \leq 40$ , r is a number satisfying  $0.88 \leq r \leq 7.2$  at %, and s is a number satisfying  $3.5 \leq s \leq 13.5$  at %; and a metallic structure including a cell phase and a cell wall phase. The cell phase has a  $\text{Th}_2\text{Zn}_{17}$  crystal phase. The cell wall phase exists to surround the cell phase. In the permanent magnet of the embodiment, a Fe concentration (C1) in the cell phase is in a range from 28 at % to 45 at %, and a difference (C1—C2) between the Fe concentration (C1) in the cell phase and a Fe concentration (C2) in the cell wall phase is larger than 10 at %.

Hereinafter, the permanent magnet of the embodiment will be described in detail. In the composition formula (1), as the element R, at least one element selected from rare-earth elements including yttrium (Y) is used. Any of the elements R brings about great magnetic anisotropy and gives a high coercive force to the permanent magnet. As the element R, at least one element selected from samarium (Sm), cerium (Ce), neodymium (Nd), and praseodymium (Pr) is preferably used, and the use of Sm is especially desirable. When 50 at % or more of the element R is Sm, it is possible to enhance performance, especially the coercive force, of the permanent magnet with good reproducibility. Further, 70 at % or more of the element R is desirably Sm.

The content p of the element R is set to a range not less than 10 at % nor more than 13.5 at %. When the content p of the element R is less than 10 at %, it is not possible to obtain a sufficient coercive force because of reasons such as the precipitation of a large amount of an  $\alpha$ -Fe phase. On the other hand, when the content p of the element R is over 13.5 at %, saturation magnetization greatly decreases. The content p of the element R is preferably set to a range of 10.2 at % to 13 at %, and more preferably a range of 10.5 at % to 12.5 at %.

Iron (Fe) is an element mainly responsible for the magnetization of the permanent magnet. When a large amount of Fe is contained, it is possible to increase saturation magnetization of the permanent magnet. However, when an excessively large amount of Fe is contained, the  $\alpha$ -Fe phase precipitates and it is difficult to obtain a later-described desired two-phase separation structure, which is liable to lower the coercive force. Therefore, the content q of Fe is set to a range not less than 28 at % nor more than 40 at %. The content q of Fe is preferably set to a range of 29 at % to 38 at %, and more preferably a range of 30 at % to 36 at %.

As the element M, at least one element selected from titanium (Ti), zirconium (Zr), and hafnium (Hf) is used. Compounding the element M makes it possible for a large coercive force to be exhibited even when the Fe concentration of the composition is high. The content r of the element

M is set to a range not less than 0.88 at % nor more than 7.2 at %. By setting the content r of the element M to 0.88 at % or more, it is possible for the permanent magnet having the composition with a high Fe concentration to exhibit a high coercive force. On the other hand, when the content r of the element M is over 7.2 at %, magnetization greatly lowers. The content r of the element M is preferably set to a range of 1.3 at % to 4.3 at %, and more preferably a range of 1.5 at % to 2.6 at %.

The element M may be any of Ti, Zr, and Hf, but preferably contains at least Zr. Especially when 50 at % or more of the element M is Zr, it is possible to further improve the effect of enhancing the coercive force of the permanent

magnet. On the other hand, Hf in the element M is especially expensive, and therefore, even when Hf is used, its amount used is preferably small. The content of Hf is preferably set to less than 20 at % of the element M.

Copper (Cu) is an element for causing the permanent magnet to exhibit a high coercive force. The content s of Cu is set to a range not less than 3.5 at % nor more than 13.5 at %. When the content s of Cu is less than 3.5 at %, it is difficult to obtain a high coercive force. When the content s of Cu is over 13.5 at %, magnetization greatly lowers. The compounding amount s of Cu is preferably set to a range of 3.9 at % to 9 at %, and more preferably a range of 4.2 at % to 7.2 at %.

Cobalt (Co) is an element not only responsible for the magnetization of the permanent magnet but also necessary for causing a high coercive force to be exhibited. Further, when a large amount of Co is contained, a Curie temperature becomes high, which improves thermal stability of the permanent magnet. When the content of Co is too small, it is not possible to sufficiently obtain these effects. However, when the content of Co is excessively large, a ratio of the Fe content relatively lowers, which deteriorates the magnetization. Therefore, the content of Co is set in consideration of the contents of the element R, the element M, and Cu so that the content of Fe satisfies the aforesaid range.

Part of Co may be substituted for by at least one element A selected from nickel (Ni), vanadium (V), chromium (Cr), manganese (Mn), aluminum (Al), gallium (Ga), niobium (Nb), tantalum (Ta), and tungsten (W). These substitution element A contributes to improvement in magnetic property, for example, the coercive force. However, the excessive substitution by the element A for Co is liable to cause the deterioration of the magnetization, and therefore, an amount of the substitution by the element A is preferably 20 at % of Co or less.

In the permanent magnet of this embodiment, the Fe concentration (C1) in the cell phase falls within the range of 28 at % to 45 at %, and the difference (C1-C2) between the Fe concentration (C1) in the cell phase and the Fe concentration (C2) in the cell wall phase is more than 10 at %. It is known that a coercive force exhibiting mechanism of a  $\text{Sm}_2\text{Co}_{17}$  type magnet is a wall pinning type, and the coercive force stems from a nano-phase separation structure generated by heat treatment. The nano-phase separation structure (two-phase separation structure) includes a cell phase having a  $\text{Th}_2\text{Zn}_{17}$  crystal phase (a crystal phase having a  $\text{Th}_2\text{Zn}_{17}$  structure/2-17 phase), and a cell wall phase formed to surround a periphery of the cell phase and having a  $\text{CaCu}_5$  crystal phase (a crystal phase having a  $\text{CaCu}_5$  structure/1-5 phase). That is, the  $\text{Sm}_2\text{Co}_{17}$  type magnet has the nano-phase separation structure in which the cell phase is demarcated by the cell wall phase.

Domain wall energy of the 1-5 phase (cell wall phase) formed to demarcate the 2-17 phase (cell phase) is larger than domain wall energy of the 2-17 phase, and this difference in the domain wall energy becomes a barrier to domain wall displacement. It is thought that, because the 1-5 phase large in the domain wall energy works as a pinning site, the domain wall pinning-type coercive force is exhibited. From this point of view, it is necessary to increase the difference in the domain wall energy between the cell phase and the cell wall phase in order to enhance the coercive force of the  $\text{Sm}_2\text{Co}_{17}$  type magnet. It has been conventionally thought that making a Cu concentration of the cell phase and a Cu concentration of the cell wall phase different from each other is effective to increase the difference in the domain wall energy.

However, when the Fe concentration of the  $\text{Sm}_2\text{Co}_{17}$  type magnet becomes high, it tends to be difficult for a high coercive force to be exhibited. One reason for this may be, for example, that it is difficult to generate the 1-5 phase being the pinning site. This is thought to be because, when the Fe concentration becomes high, a hetero-phase (Cu-M rich phase) in which the concentrations of Cu and the element M are high is easily generated and a Cu concentration in a main phase ( $\text{TbCu}_7$  crystal phase/1-7 phase) being a precursor phase of the two-phase separation structure lowers, so that the phase separation of the main phase to the cell phase and the cell wall phase is difficult to progress.

Another possible reason why the coercive force of the  $\text{Sm}_2\text{Co}_{17}$  type magnet becomes small is that in accordance with an increase in the Fe concentration, the difference in the domain wall energy between the cell phase and the cell wall phase becomes small, so that the effect of the pinning of the domain wall by the cell wall phase decreases. It has been thought that the difference in the domain wall energy stems from a ratio of constituent elements of the cell phase and the cell wall phase, and it is especially important that Cu is condensed in the cell wall phase to form a potential well. Therefore, it has been thought to be effective to make the cell phase and the cell wall phase different in the Cu concentration by a certain degree as described above. However, studies by the present inventors have made it clear that, though this applies to a conventional  $\text{Sm}_2\text{Co}_{17}$  type magnet but is not true in a composition range where the Fe concentration is high.

In  $\text{Sm}_2\text{Co}_{17}$  type magnets with a Fe concentration of about 20 at % that have been reported so far, the Cu concentration difference between the cell wall phase and the cell phase is about 10 at % to about 20 at %. On the other hand, as a result of the investigation by the present inventors, approximately the same degree of the Cu concentration difference has been confirmed also in  $\text{Sm}_2\text{Co}_{17}$  type magnets having a composition with a Fe concentration of 28 at % or more. Nevertheless, a sufficient coercive force has not been obtained in the  $\text{Sm}_2\text{Co}_{17}$  type magnets having a high Fe concentration. Careful observation of microstructures of these magnets have made it clear that the Fe concentration difference between the cell phase and the cell wall phase in magnets having a high Fe concentration is smaller than or about equal to that of conventional magnets. This indicates that Cu is condensed in the cell phase but the diffusion of Fe to the cell phase is insufficient.

In the permanent magnet of this embodiment, the Fe concentration (C1) in the cell phase falls within the range of 28 at % to 45 at %, and the difference between the Fe concentration (C1) in the cell phase and the Fe concentration (C2) in the cell wall phase is larger than 10 at %. Studies by the present inventors have made it clear that the Fe concentration difference between the cell phase and the cell wall phase also influences the difference in the domain wall energy in the composition range in which the Fe concentration is high. When the Fe concentration difference (C1-C2) between the cell phase and the cell wall phase is larger than 10 at %, the difference in the domain wall energy between the cell phase and the cell wall phase is large. Therefore, it is possible to enhance the coercive force of the  $\text{Sm}_2\text{Co}_{17}$  type magnet having a high Fe concentration.

Further, that Fe is condensed in the cell phase means that the mutual diffusion of Cu and Fe is sufficiently progressing. Therefore, increasing the Fe concentration difference between the cell phase and the cell wall phase also increases the Cu concentration difference between the cell phase and

the cell wall phase. Accordingly, the difference in the domain wall energy between the cell phase and the cell wall phase also becomes large, which can enhance the coercive force of the  $\text{Sm}_2\text{Co}_{17}$  type magnet having a high Fe concentration. It has been conventionally thought that Cu and Fe mutually diffuse, but it is what the present inventors have newly found that the Fe concentration difference between the cell phase and the cell wall phase influences the difference in the domain wall energy, and as a result influences the coercive force.

The Fe concentration (C1) in the cell phase is set to 28 at % or more in order to enhance the magnetization of the permanent magnet. In order to increase the Fe concentration difference between the cell phase and the cell wall phase, the Fe concentration (C1) in the cell phase is preferably 28.5 at % or more, and more preferably 29 at % or more. Such a Fe concentration (C1) of the cell phase can be realized by the sufficient diffusion of Fe into the cell phase. The Fe concentration difference between the cell phase and the cell wall phase is preferably 12 at % or more, and more preferably 14 at % or more.

The Fe concentration (C2) in the cell wall phase is adjusted so as to be different from the Fe concentration (C1) in the cell phase by more than 10 at %. The Cu concentration of the cell wall phase is preferably 1.2 times the Cu concentration of the cell phase, and more preferably twice or more. This makes it possible for the cell wall phase to fully function as the pinning site of the domain wall. A typical example of the cell wall phase is the 1-5 phase, but the cell wall phase is not limited to this. If the Fe concentration difference and the Cu concentration difference between the cell phase and the cell wall phase are sufficiently large, the cell wall phase functions as the pinning site of the domain wall. The cell wall phase only needs to be such a phase. Besides the 1-5 phase, examples of the cell wall phase are the 1-7 phase being a high-temperature phase (structure before the phase separation), the precursor phase of the 1-5 phase that is generated in an initial stage of the two-phase separation of the 1-7 phase, and the like.

Incidentally, in order to fully progress the mutual diffusion of Fe and Cu to realize the aforesaid Fe concentration difference between the cell phase and the cell wall phase in the permanent magnet made of a sintered compact having the composition expressed by the composition formula (1), it is effective to increase the density of the sintered compact to increase a diffusible area. However, since Sm—Co-based magnetic powder (alloy powder) having a high Fe concentration is low in sinterability, it is difficult to obtain a high density of the sintered compact. When the Fe concentration of the alloy powder is high, a hetero-phase in which the concentrations of Cu and the element M are high is likely to be generated, and it is thought that this hetero-phase worsens sinterability. In order to progress the mutual diffusion of Fe and Cu, it is important to suppress the generation of the hetero-phase to improve sinterability of the magnetic powder (alloy, powder) having a high Fe concentration. Examples of the hetero-phase mentioned here are Zr and Cu-rich phases such as a 2-7 phase in which a ratio of the element R such as Sm to transition metal elements such as Co and Fe is 2 to 7, a 1-13 phase in which the ratio is 1 to 13, and so on.

The sintering of the Sm—Co based magnetic powder (alloy powder) is generally performed in an inert gas atmosphere such as Ar gas or in a vacuum atmosphere. The sintering in the inert gas atmosphere has a merit of being capable of suppressing the evaporation of Sm having a high vapor pressure to make composition deviation difficult to

occur. However, in the inert gas atmosphere, it is difficult to avoid the generation of the hetero-phase. Moreover, the inert gas such as the Ar gas remains in pores to make the pores difficult to disappear, which makes it difficult to increase the density of the sintered compact. On the other hand, it has been made clear that the sintering in the vacuum atmosphere can suppress the generation of the hetero-phase. However, an evaporation amount of Sm having a high vapor pressure becomes large in the vacuum atmosphere, which makes it difficult to control the composition of the sintered compact to an alloy composition suitable as the permanent magnet.

As a solution to such problems, it is effective to perform a final sintering step (main sintering step) in the inert gas atmosphere of Ar gas or the like after a pre-process step (temporary sintering step) in the vacuum atmosphere is performed. By employing such a sintering step having the pre-process step in the vacuum atmosphere and the main sintering step in the inert gas atmosphere, it is possible to suppress the evaporation of Sm or the like having a high vapor pressure while suppressing the generation of the hetero-phase in which the concentrations of Cu and the element M are high. Therefore, it is possible to obtain the sintered compact with a high density and a small composition deviation when the magnetic powder (alloy powder) having a high Fe concentration is used. By obtaining the sintered compact with a high density and a small composition deviation, it is possible to fully progress the mutual diffusion of Fe and Cu in later solution treatment step and aging step. This makes it possible to increase the Fe concentration difference between the cell phase and the cell wall phase.

When the magnetic powder (alloy powder) having a Fe concentration of about 20 at % is sintered, setting a temperature of the temporary sintering step lower than a temperature of the main sintering step by a certain degree is effective for increasing the density. On the other hand, when the magnetic powder (alloy powder) having a Fe concentration of 28 at % or more is sintered, it is preferable to keep the vacuum atmosphere until the temperature becomes as close to the temperature of the main sintering step as possible. Further, keeping the vacuum atmosphere until the temperature of the main sintering is reached is also effective. In this case as well, by changing to the inert gas at the same time when the temperature of the main sintering is reached, it is possible to suppress the evaporation of Sm or the like in the sintered compact. A reason why it is preferable to keep the vacuum atmosphere until the temperature becomes close to the temperature of the main sintering when the composition is in the range having a high Fe concentration is thought to be that keeping the vacuum atmosphere until the temperature becomes as high as possible makes it possible to more effectively suppress the generation of the hetero-phase. Concrete conditions in the sintering step of the magnetic powder (alloy powder) will be described in detail later.

By subjecting the aforesaid high-density sintered compact to the solution treatment and the aging, it is possible to increase the Fe concentration difference between the cell phase and the cell wall phase with good reproducibility. This makes it possible to enhance the coercive force of the Sm—Co based magnet having the composition with a high Fe concentration. Specifically, the permanent magnet of this embodiment has an enhanced coercive force owing to the Fe concentration difference between the cell phase and the cell wall phase while achieving improved magnetization owing to the Fe concentration of 28 at % or more, and realizes both a high coercive force and high magnetization in the Sm—Co

based magnet. The coercive force of the permanent magnet of the embodiment is preferably 800 kA/m or more, and the residual magnetization is preferably 1.15 T or more.

The density of the sintered compact of the Sm—Co based magnetic powder (alloy powder) is preferably  $8.2 \times 10^3$  kg/m<sup>3</sup> or more from a practical point of view. By realizing such a density of the sintered compact, it is possible to fully progress the mutual diffusion of Fe and Cu in the solution treatment step and the aging step to increase the Fe concentration difference between the cell phase and the cell wall phase. The permanent magnet of the embodiment is preferably a sintered magnet that includes a sintered compact including the composition expressed by the composition formula (1) and the metallic structure having the cell phase and the cell wall phase, wherein the density of the sintered compact is  $8.2 \times 10^3$  kg/m<sup>3</sup> or more.

In the permanent magnet of the embodiment, it is possible to observe the metallic structure having a cell-like structure by using a transmission electron microscope (TEM). The TEM observation is preferably conducted with a magnification of 100 k to 200 k times. In the permanent magnet made of the sintered compact oriented by a magnetic field, a cross section including a c-axis of the 2-17 phase being the cell phase is preferably observed with TEM. The cell wall phase is a region having a Cu concentration 1.2 times that of the cell phase or more. Composition analysis of the elements such as Fe and Cu in the cell phase and the cell wall phase is conducted with, for example, a TEM-energy dispersive X-ray spectroscopy (TEM-EDX). The TEM-EDX observation is conducted for the interior of the sintered compact.

The measurement of the interior of the sintered compact means as follows. First, the composition is measured in a surface portion and the interior of a cross section cut at a center portion of the longest side in a surface having the largest area, perpendicularly to the side (perpendicularly to a tangent of the center portion in a case of a curve). Measurement points are as follows. Reference lines 1 drawn from  $\frac{1}{2}$  positions of respective sides in the aforesaid cross section as starting points up to end portions toward an inner side perpendicularly to the sides and reference lines 2 drawn from centers of respective corners as starting points up to end portions toward the inner side at  $\frac{1}{2}$  positions of interior angles of the corner portions are provided, and 1% positions of the lengths of the reference lines from the starting points of these reference lines 1, 2 are defined as the surface portion and 40% positions are defined as the interior. Note that, when the corner portions have curvature because of chamfering or the like, points of intersection of extensions of adjacent sides are defined as the end portions (centers of the corner portions). In this case, the measurement points are positions determined not based on the points of intersection but based on portions in contact with the reference lines.

When the measurement points are decided as above, in a case where the cross section is, for example, a quadrangular, the number of the reference lines is totally eight, with the four reference lines 1 and the four reference lines 2, and the number of the measurement points is eight in each of the surface portion and the interior. In this embodiment, the eight points in each of the surface and the interior all preferably have the composition within the aforesaid range, but at least four points or more in each of the surface portion and the interior need to have the composition within the aforesaid range. In this case, a relation between the surface portion and the interior of one reference line is not defined. The TEM observation is conducted after an observation surface of the interior of the sintered compact thus defined is smoothed by polishing. The points of the TEM-EDX

observation are arbitrary 20 points in the cell phase and the cell wall phase, and an average value of measurement values except the maximum value and the minimum value of the measurement values at these points is found, and this average value is set as the concentration of each element.

The permanent magnet of this embodiment is fabricated as follows, for instance. First, alloy powder containing predetermined amounts of elements is fabricated. The alloy powder is prepared by grinding an alloy ingot obtained through the forging of molten metal by an arc melting method or a high-frequency melting method. The alloy powder may be prepared by fabricating an alloy thin strip in a flake form by a strip cast method and thereafter grinding the alloy thin strip. In the strip cast method, it is preferable that the alloy molten metal is tiltingly injected to a chill roll rotating at a 0.1 m/second to 20 m/second circumferential speed and a thin strip with a 1 mm thickness or less is continuously obtained. When the circumferential speed of the chill roll is less than 0.1 m/second, a composition variation is likely to occur in the thin strip, and when the circumferential speed is over 20 m/second, crystal grains become fine to a single domain size or less and a good magnetic property cannot be obtained. The circumferential speed of the chill roll preferably falls within a range of 0.3 m/second to 15 m/second, and more preferably within a range of 0.5 m/second to 12 m/second.

Other examples of the method of preparing the alloy powder are a mechanical ironing method, a mechanical grinding method, a gas atomization method, a reduction diffusion method, and the like. The alloy powder prepared by any of these methods may be used. The alloy powder thus obtained or the alloy before being ground may be heat-treated for homogenization when necessary. A jet mill or a ball mill is used for grinding the flake or the ingot. The grinding is preferably performed in an inert gas atmosphere or an organic solvent in order to prevent oxidization of the alloy powder.

Next, the alloy powder is filled in a mold installed in an electromagnet or the like and is press-formed while a magnetic field is applied. Consequently, a compression-molded body whose crystal axes are oriented is fabricated. By sintering the compression-molded body under appropriate conditions, it is possible to obtain a sintered compact having a high density. The sintering step of the compression-molded body preferably includes the pre-process step in the vacuum atmosphere and the main sintering step in the inert gas atmosphere as previously described. A main sintering temperature  $T_s$  is preferably 1215° C. or lower. When the Fe concentration is high, it is expected that a melting point lowers, and therefore, Sm or the like easily evaporates when the main sintering temperature  $T_s$  is too high. The main sintering temperature  $T_s$  is more preferably 1205° C. or lower, and still more preferably 1195° C. or lower. However, in order to increase the density of the sintered compact, the main sintering temperature  $T_s$  is preferably 1170° C. or higher, and still more preferably 1180° C. or higher.

In the main sintering step in the inert gas atmosphere, the sintering time at the aforesaid main sintering temperature  $T_s$  is preferably 0.5 hour to 15 hours. This makes it possible to obtain a dense sintered compact. When the sintering time is less than 0.5 hour, the density of the sintered compact becomes uneven. When the sintering time is over 15 hours, Sm or the like in the alloy powder evaporates, which is liable to make it impossible to obtain a good magnetic property. The sintering time is more preferably one hour to ten hours,

and still more preferably one hour to four hours. The main sintering step is performed in the inert gas atmosphere of Ar gas or the like.

As previously described, in order to turn the compression-molded body of the alloy powder having a high Fe concentration to the high-density sintered compact, the pre-process step is preferably performed in the vacuum atmosphere prior to the main sintering step. Further, it is preferable that the vacuum atmosphere is kept until the temperature becomes close to the main sintering temperature. Concretely, in order for the sintered compact to have a density of  $8.2 \times 10^3$  kg/m<sup>3</sup> or more, the temperature T [°C.] at the time of the change from the vacuum atmosphere to the inert gas atmosphere (pre-process temperature) preferably falls within a temperature range not lower than a temperature that is lower than the main sintering temperature Ts [°C.] by 50° C. (Ts-50° C.) nor higher than the main sintering temperature Ts (Ts-50° C.  $\leq$  T  $\leq$  Ts). When the atmosphere change temperature T is lower than the main sintering temperature Ts by more than 50° C. (T < Ts-50° C.), it might not be possible to sufficiently increase the density of the sintered compact. Moreover, the hetero-phase existing in the compression-molded body or the hetero-phase generated at the time of the temperature increase in the sintering step remains even after the main sintering step, which is liable to lower the magnetization.

When the atmosphere change temperature T is too lower than the main sintering temperature Ts, it is not possible to fully obtain the effect of suppressing the generation of the hetero-phase in the pre-process step in the vacuum atmosphere. Accordingly, it is not possible to increase the density of the sintered compact, which lowers both the magnetization and the coercive force. The atmosphere change temperature T is more preferably equal to or higher than a temperature that is lower than the main sintering temperature Ts by 40° C. (Ts-40° C.), and still more preferably equal to or higher than a temperature that is lower than the main sintering temperature Ts by 30° C. (Ts-30° C.). However, when the process temperature T in the vacuum atmosphere is higher than the main sintering temperature Ts, Sm evaporates to deteriorate the magnetic property, and therefore, the atmosphere change temperature T is set to the main sintering temperature Ts or lower. The change from the vacuum atmosphere to the inert gas atmosphere may take place at the same time when the main sintering temperature Ts is reached.

The vacuum atmosphere (degree of vacuum) in the pre-process step is preferably set to  $9 \times 10^{-2}$  Pa or less. When the degree of vacuum of the pre-process step is over  $9 \times 10^{-2}$  Pa, an oxide of the element R such as Sm is liable to be excessively formed. By setting the degree of vacuum in the pre-process step to  $9 \times 10^{-2}$  Pa or less, it is possible to more effectively obtain the effect of increasing the Fe concentration difference between the cell phase and the cell wall phase. The degree of vacuum of the pre-process step is more preferably  $5 \times 10^{-2}$  Pa or less, and still more preferably  $1 \times 10^{-2}$  Pa or less.

Further, it is also effective to keep the vacuum atmosphere for a predetermined time at the time of the change from the vacuum atmosphere to the inert gas atmosphere. This makes it possible to further promote the density increase of the sintered compact and also improve the effect of increasing the Fe concentration difference between the cell phase and the cell wall phase. The retention time in the vacuum atmosphere is preferably set based on the composition of the alloy powder (magnetic powder), especially the composition of the element R such as Sm. Concretely, the retention time in the vacuum atmosphere is preferably set equal to or longer

than a time Y [minute] satisfying the following expression (2) based on the concentration (p1 [at %]) of the element R in the alloy powder (magnetic powder).

$$Y = -5p_1 + 62 \quad (2)$$

By changing from the vacuum atmosphere to the inert gas atmosphere after keeping the vacuum atmosphere for the time Y or more and performing the main sintering step, it is possible to more effectively increase the density of the sintered compact when the alloy powder in which the Fe concentration is high and the concentration of the element R such as Sm is low is used. The time Y is preferably shorter than a main sintering time. When the time Y is too long, an evaporation amount of the element R such as Sm is liable to increase. In a case of a composition range where the concentration p1 of the element R is high, a value of Y sometimes become minus. In the case of such a composition range that the value of Y becomes minus, a relatively high density is easily obtained, but even in such a case, by keeping the vacuum atmosphere for one minute or more, it is possible to stably increase the density of the sintered compact. When the atmosphere change temperature T is lower than the main sintering temperature Ts, the atmosphere change temperature T is kept for a predetermined time. When the atmosphere change temperature T is set to a temperature equal to the main sintering temperature Ts, the temperature is increased up to the main sintering temperature Ts after the temperature lower than the main sintering temperature Ts is kept for a predetermined time, and the atmospheres are changed.

The measurement of the concentration p1 of the element R in the alloy powder (magnetic powder) used for fabricating the sintered compact is preferably performed for the powder finely ground by the jet mill or the ball mill. The measurement of the concentration p1 of the element R may be performed for the roughly ground powder not yet finely ground. The concentration p1 of the element R can be found by an inductively coupled plasma (ICP) emission spectrochemical analysis method. The measurement by the ICP emission spectrochemical analysis method is performed for the target powder ten times, and an average value of measurement values excluding the maximum value and the minimum value of these measurement values is defined as the concentration p1 of the element R. When a mixture of two kinds of more of raw material powders different in composition is used, not the concentration of the element R found from the compositions of the respective raw material powders is measured, but the concentration p1 of the element R is measured after the two kinds or more of the raw material powders are mixed.

The main sintering step in the inert gas atmosphere follows the pre-process step in the vacuum atmosphere. In this case, the vacuum atmosphere is changed to the inert gas atmosphere at the same time when the main sintering temperature Ts is reached, the vacuum atmosphere is changed to the inert gas atmosphere when the atmosphere change temperature T which is equal to or higher than the temperature lower than the main sintering temperature Ts by 50° C. (Ts-50° C.) is reached, or the vacuum atmosphere is changed to the inert gas atmosphere after the atmosphere change temperature T is kept for a predetermined time. The pre-process step in the vacuum atmosphere and the main sintering step in the inert gas atmosphere may be performed as separate steps. In this case, the temperature is increased up to the atmosphere change temperature (pre-process temperature) T in the vacuum atmosphere, and when necessary, after this temperature is kept for a predetermined time,

## 11

cooling is performed. Next, after the vacuum atmosphere is changed to the inert gas atmosphere, the temperature is increased up to the main sintering temperature  $T_s$  and the main sintering step is performed.

Next, the solution treatment and the aging are applied to the obtained sintered compact to control the crystal structure. The solution treatment is preferably 0.5-hour to eight-hour heat treatment at the temperature range of 1100°C. to 1190°C. in order to obtain the 1-7 phase being the precursor of the phase separation structure. When the temperature is lower than 1100°C. or is over 1190°C., a ratio of the 1-7 phase in a sample having undergone the solution treatment is small and a good magnetic property is not obtained. The temperature of the solution treatment more preferably falls within a range of 1120°C. to 1180°C., and more preferably within a range of 1120°C. to 1170°C.

When the solution treatment time is less than 0.5 hour, the constituent phase is likely to be uneven, which is liable to make it impossible to obtain a more sufficient density. When the solution treatment time is over eight hours, the element R such as Sm in the sintered compact evaporates, which is liable to make it impossible to obtain a good magnetic property. The solution treatment time more preferably falls within a range of one hour to eight hours, and more preferably within a range of one hour to four hours. For the prevention of oxidation, the solution treatment is performed in the vacuum atmosphere or the inert gas atmosphere of Ar gas or the like.

Next, the aging is applied to the sintered compact having undergone the solution treatment. The aging is treatment to control the crystal structure to enhance the coercive force of the magnet. In the aging, it is preferable that after the temperature is kept at 700°C. to 900°C. for 0.5 hour to 80 hours, the temperature is gradually decreased to 400°C. to 650°C. at a cooling rate of 0.2°C./minute to 2°C./minute, and the temperature is subsequently decreased to room temperature. The aging may be performed by two-stage heat treatment. The aforesaid heat treatment is the first stage and after the temperature is gradually decreased to 400°C. to 650°C., the second-stage heat treatment is subsequently performed. After the temperature of the second-stage heat treatment is kept for a certain time, the temperature is decreased to room temperature by furnace cooling. In order to prevent oxidation, the aging is preferably performed in the vacuum atmosphere or the inert gas atmosphere of Ar gas or the like.

When the aging temperature is lower than 700°C. or is over 900°C., it is not possible to obtain a uniform mixed structure of the cell phase and the cell wall phase, which is liable to deteriorate the magnetic property of the permanent magnet. The aging temperature is more preferably 750°C. to 880°C., and still more preferably 780°C. to 850°C. When the aging time is less than 0.5 hour, the precipitation of the cell wall phase from the 1-7 phase might not be fully completed. On the other hand, when the retention time is over 80 hours, the thickness of the cell wall phase becomes large, so that a volume fraction of the cell phase lowers and crystal grains roughen, which is liable to make it impossible to obtain a good magnetic property. The aging time is more preferably four hours to sixty hours, and still more preferably eight hours to forty hours.

When the cooling rate of the aging treatment is less than 0.2°C./minute, the thickness of the cell wall phase becomes large, so that a volume fraction of the cell phase lowers or crystal grains roughen, which is liable to make it impossible to obtain a good magnetic property. When the cooling rate after the aging heat treatment is over 2°C./minute, it is not

## 12

possible to obtain a uniform mixed structure of the cell phase and the cell wall phase, which is liable to deteriorate the magnetic property of the permanent magnet. The cooling rate after the aging heat treatment is more preferably set to a range of 0.4°C./minute to 1.5°C./minute, and still more preferably a range of 0.5°C./minute to 1.3°C./minute.

Note that the aging is not limited to the two-stage heat treatment but may be heat treatment in more multiple stages, and it is also effective to perform multi-stage cooling. As a 10 pre-process of the aging, it is also effective to perform preliminary aging at a temperature lower than that of the aging for a short time. This is expected to improve squareness of a magnetization curve. By setting the temperature of the preliminary aging to 650°C. to 790°C., the treatment 15 time to 0.5 hour to four hours, and the gradual cooling rate after the aging to 0.5°C./minute to 1.5°C./minute, the improvement in the squareness of the permanent magnet is expected.

The permanent magnet of this embodiment is usable in 20 various kinds of motors and power generators. The permanent magnet of the embodiment is also usable as a stationary magnet and a variable magnet of a variable magnetic flux motor and a variable magnetic flux power generator. Various kinds of motors and power generators are structured by the 25 use of the permanent magnet of this embodiment. When the permanent magnet of this embodiment is applied to a variable magnetic flux motor, arts disclosed in Japanese Patent Application Laid-open No. 2008-29148 and Japanese Patent Application Laid-open No. 2008-43172 are applicable 30 as a structure and a drive system of the variable magnetic flux motor.

Next, a motor and a power generator of embodiments will be described with reference to the drawings. FIG. 1 shows a permanent magnet motor according to an embodiment. In 35 the permanent magnet motor 1 shown in FIG. 1, a rotor (rotating part) 3 is disposed in a stator (stationary part) 2. In an iron core 4 of the rotor 3, the permanent magnets 5 of the embodiment are disposed. Based on the properties and so on of the permanent magnets of the embodiment, it is possible 40 to realize efficiency enhancement, downsizing, cost reduction, and so on of the permanent magnet motor 1.

FIG. 2 shows a variable magnetic flux motor according to an embodiment. In the variable magnetic flux motor 11 shown in FIG. 2, a rotor (rotating part) 13 is disposed in a stator (stationary part) 12. In an iron core 14 of the rotor 13, the permanent magnets of the embodiment are disposed as stationary magnets 15 and variable magnets 16. Magnetic flux density (flux quantum) of the variable magnets 16 is variable. The variable magnets 16 are not influenced by a Q-axis current because their magnetization direction is orthogonal to a Q-axis direction, and can be magnetized by a D-axis current. In the rotor 13, a magnetized winding (not shown) is provided. When a current is passed through the magnetized winding from a magnetizing circuit, its magnetic field acts directly on the variable magnets 16.

According to the permanent magnet of the embodiment, it is possible to obtain a suitable coercive force in the stationary magnets 15. When the permanent magnets of the embodiment are applied to the variable magnets 16, the coercive force is controlled to, for example, a 100 kA/m to 500 kA/m range by changing the various conditions (aging condition and so on) of the aforesaid manufacturing method. In the variable magnetic flux motor 11 shown in FIG. 2, the permanent magnets of the embodiment are usable as both of the stationary magnets 15 and the variable magnets 16, but the permanent magnets of the embodiment may be used as either of the magnets. The variable magnetic flux motor 11

is capable of outputting a large torque with a small device size and thus is suitable for motors of hybrid vehicles, electric vehicles, and so on whose motors are required to have a high output and a small size.

FIG. 3 shows a power generator according to an embodiment. The power generator 21 shown in FIG. 3 includes a stator (stationary part) 22 using the permanent magnet of the embodiment. A rotor (rotating part) 23 disposed inside the stator (stationary part) 22 is connected via a shaft 25 to a turbine 24 provided at one end of the power generator 21. The turbine 24 rotates by an externally supplied fluid, for instance. Incidentally, instead of the turbine 24 rotating by the fluid, it is also possible to rotate the shaft 25 by the transmission of dynamic rotation such as regenerative energy of a vehicle. As the stator 22 and the rotor 23, various kinds of generally known structures are adoptable.

The shaft 25 is in contact with a commutator (not shown) disposed on the rotor 23 opposite the turbine 24, and an electromotive force generated by the rotation of the rotor 23 is boosted to system voltage to be transmitted as an output of the power generator 21 via an isolated phase bus and a traction transformer (not shown). The power generator 21 may be either of an ordinary power generator and a variable magnetic flux power generator. Incidentally, the rotor 23 is electrically charged due to an axial current accompanying static electricity from the turbine 24 and the power generation. Therefore, the power generator 21 includes a brush 26 for discharging the charged electricity of the rotor 23.

Next, examples and their evaluation results will be described.

#### Examples 1, 2

After raw materials were weighed and mixed at a predetermined ratio, the resultant was arc-melted in an Ar gas atmosphere, whereby an alloy ingot was fabricated. After the alloy ingot was heat-treated at 1180°C. for four hours, it was roughly ground and then finely ground by a jet mill, whereby alloy powder as raw material powder of a permanent magnet was prepared. The alloy powder was press-formed in a magnetic field, whereby a compression-molded body was fabricated.

Next, the compression-molded body of the alloy powder was disposed in a chamber of a firing furnace, and the chamber was vacuum-exhausted until its degree of vacuum became  $9.0 \times 10^{-3}$  Pa. In this state, a temperature in the chamber was raised up to 1160°C., and after this temperature was kept for five minutes, Ar gas was led into the chamber. The temperature in the chamber set to the Ar atmosphere was raised up to 1195°C., and this temperature was kept for two hours and the main sintering was performed. The pre-process temperature (atmosphere change temperature) T in the vacuum in the examples 1, 2 was set to 1160°C. which is lower than 1195°C. being the main sintering temperature Ts by 35°C. Sintering conditions are shown in Table 2.

Subsequently to the main sintering step, the sintered compact was kept at 1145°C. for four hours and was subjected to solution treatment. Next, after the sintered compact having undergone the solution treatment was kept at 750°C. for two hours, it was gradually cooled to room temperature and was further kept at 815°C. for thirty hours. After the sintered compact having undergone aging under such conditions was gradually cooled to 400°C., it was cooled in the furnace to room temperature, whereby a desired sintered magnet was obtained. The composition of the sintered magnet is as shown in Table 1. Composition

analysis of the magnet was conducted by the ICP method. Following the aforesaid method, a density of the sintered compact, a Fe concentration (C1) of a cell phase, and a Fe concentration difference (C1-C2) between the cell phase and a cell wall phase were measured. Further, magnetic properties of each of the sintered magnets were evaluated by a BH tracer and a coercive force and residual magnetization were measured. The results are shown in Table 3.

Note that the composition analysis by the ICP method was done in the following procedure. First, a predetermined amount of a sample ground in a mortar is weighed and is put into a quartz beaker. A mixed acid (containing nitric acid and hydrochloric acid) is put into the quartz beaker, which is heated to about 140°C. on a hotplate, whereby the sample is completely melted. After it is left standing to cool, it is transferred to a PFA volumetric flask and is subjected to an isovolumetric process to be a sample solution. Quantities of components of such a sample solution were determined by a calibration curve method with the use of an ICP emission spectrochemical analyzer. As the ICP emission spectrochemical analyzer, SPS4000 (trade name) manufactured by SII Nano Technology Inc. was used

#### Example 3

After raw materials were weighed and mixed at a predetermined ratio, the resultant was high-frequency melted in an Ar gas atmosphere, whereby an alloy ingot was fabricated. After the alloy ingot was heat-treated at 1175°C. for two hours, it was roughly ground and then finely ground by a jet mill, whereby alloy powder as raw material powder of a permanent magnet was prepared. The alloy powder was press-formed in a magnetic field, whereby a compression-molded body was fabricated.

Next, the compression-molded body of the alloy powder was disposed in a chamber of a firing furnace, and the chamber was vacuum-exhausted until its degree of vacuum became  $9.0 \times 10^{-3}$  Pa. In this state, a temperature in the chamber was raised up to 1185°C., and after this temperature was kept for one minute, Ar gas was led into the chamber. The temperature in the chamber set to the Ar atmosphere was raised up to 1195°C., and this temperature was kept for three hours and the main sintering was performed. Subsequently, the sintered compact was kept at 1140°C. for six hours and was subjected to solution treatment.

Next, after the sintered compact having undergone the solution treatment was kept at 760°C. for 1.5 hours, it was gradually cooled to room temperature. Subsequently, after it was kept at 800°C. for 45 hours, it was gradually cooled to 400°C., and was further cooled in a furnace to room temperature, whereby a desired sintered magnet was obtained. The composition of the sintered magnet is as shown in Table 1. Regarding the obtained sintered magnet, a density of a sintered compact, a Fe concentration (C1) of a cell phase, a Fe concentration difference (C1-C2) between the cell phase and a cell wall phase, a coercive force, and residual magnetization were measured in the same manner as in the example 1. The measurement results are shown in Table 3.

#### Example 4

After raw materials were weighed and mixed at a predetermined ratio, the resultant was high-frequency melted in an Ar gas atmosphere, whereby an alloy ingot was fabricated. After the alloy ingot was heat-treated at 1180°C. for

15

one hour, it was roughly ground and then finely ground by a jet mill, whereby alloy powder as raw material powder of a permanent magnet was prepared. The alloy powder was press-formed in a magnetic field, whereby a compression-molded body was fabricated.

Next, the compression-molded body of the alloy powder was disposed in a chamber of a firing furnace, and the chamber was vacuum-exhausted until its degree of vacuum became  $8.0 \times 10^{-3}$  Pa. In this state, a temperature in the chamber was raised up to  $1180^\circ$  C., and after this temperature was kept for twenty minutes, Ar gas was led into the chamber. The temperature in the chamber set to the Ar atmosphere was raised up to  $1205^\circ$  C., and this temperature was kept for two hours and main sintering was performed. Subsequently, the sintered compact was kept at  $1150^\circ$  C. for eight hours and was subjected to solution treatment.

Next, after the sintered compact having undergone the solution treatment was kept at  $730^\circ$  for three hours, it was gradually cooled to room temperature. Subsequently, after it was kept at  $810^\circ$  C. for 35 hours, it was gradually cooled to  $450^\circ$  C., and was further cooled in a furnace to room temperature, whereby a desired sintered magnet was obtained. The composition of the sintered magnet is as shown in Table 1. Regarding the obtained sintered magnet, a density of a sintered compact, a Fe concentration (C1) of a cell phase, a Fe concentration difference (C1-C2) between the cell phase and a cell wall phase, a coercive force, and residual magnetization were measured in the same manner as in the example 1. The measurement results are shown in Table 3.

#### Example 5

After raw materials were weighed and mixed at a predetermined ratio, the resultant was high-frequency melted in an Ar gas atmosphere, whereby an alloy ingot was fabricated. After the alloy ingot was heat-treated at  $1180^\circ$  C. for one hour, it was roughly ground and then finely ground by a jet mill, whereby alloy powder as raw material powder of a permanent magnet was prepared. The alloy powder was press-formed in a magnetic field to fabricate a compression-molded body.

Next, the compression-molded body of the alloy powder was disposed in a chamber of a firing furnace, and the chamber was vacuum-exhausted until its degree of vacuum became  $8.5 \times 10^{-3}$  Pa. In this state, a temperature in the chamber was raised up to  $1180^\circ$  C., and after this temperature was kept for one minute, Ar gas was led into the chamber. The temperature in the chamber set to the Ar atmosphere was raised up to  $1198^\circ$  C., and this temperature was kept for three hours and main sintering was performed. Subsequently, the sintered compact was kept at  $1140^\circ$  C. for four hours and was subjected to solution treatment.

Next, after the sintered compact having undergone the solution treatment was kept at  $750^\circ$  for two hours, it was gradually cooled to room temperature. Subsequently, after it was kept at  $820^\circ$  C. for 46 hours, it was gradually cooled to  $350^\circ$  C., and was further cooled in a furnace to room temperature, whereby a desired sintered magnet was obtained. The composition of the sintered magnet is as shown in Table 1. Regarding the obtained sintered magnet, a density of a sintered compact, a Fe concentration (C1) of a cell phase, a Fe concentration difference (C1-C2) between the cell phase and a cell wall phase, a coercive force, and

16

residual magnetization were measured in the same manner as in the example 1. The measurement results are shown in Table 3.

#### Example 6

Alloy powder having the same composition as that of the example 5 was press-formed in a magnetic field, whereby a compression-molded body was fabricated. This compression-molded body was disposed in a chamber of a firing furnace, and the chamber was vacuum-exhausted until its degree of vacuum became  $8.5 \times 10^{-3}$  Pa. In this state, a temperature in the chamber was raised up to  $1190^\circ$ , and after this temperature was kept for one minute, Ar gas was led into the chamber. The temperature in the chamber set to the Ar atmosphere was raised up to  $1198^\circ$  C., and this temperature was kept for three hours and main sintering was performed. Subsequently, solution treatment and aging were performed under the same conditions as those of the example 5, whereby a desired sintered magnet was obtained. The composition of the sintered magnet is as shown in Table 1. Regarding the obtained sintered magnet, a density of a sintered compact, a Fe concentration (C1) of a cell phase, a Fe concentration difference (C1-C2) between the cell phase and a cell wall phase, a coercive force, and residual magnetization were measured in the same manner as in the example 1. The measurement results are shown in Table 3.

#### Example 7

Alloy powder having the same composition as that of the example 5 was press-formed in a magnetic field, whereby a compression-molded body was fabricated. This compression-molded body was disposed in a chamber of a firing furnace, and the chamber was vacuum-exhausted until its degree of vacuum became  $8.5 \times 10^{-3}$  Pa. In this state, a temperature in the chamber was raised up to  $1155^\circ$  C., and after this temperature was kept for one minute, Ar gas was led into the chamber. The temperature in the chamber set to the Ar atmosphere was raised up to  $1198^\circ$  C., and this temperature was kept for three hours and the main sintering was performed. Next, solution treatment and aging were performed under the same conditions as those of the example 5, whereby a desired sintered magnet was obtained. The composition of the sintered magnet is as shown in Table 1. Regarding the obtained sintered magnet, a density of a sintered compact, a Fe concentration (C1) of a cell phase, a Fe concentration difference (C1-C2) between the cell phase and a cell wall phase, a coercive force, and residual magnetization were measured in the same manner as in the example 1. The measurement results are shown in Table 3.

#### Example 8

Alloy powder having the same composition as that of the example 2 was press-formed in a magnetic field, whereby a compression-molded body was fabricated. This compression-molded body was disposed in a chamber of a firing furnace, and the chamber was vacuum-exhausted until its degree of vacuum became  $2.8 \times 10^{-3}$  Pa. In this state, a temperature in the chamber was raised up to  $1160^\circ$  C., and after this temperature was kept for five minutes, Ar gas was led into the chamber. The temperature in the chamber set to the Ar atmosphere was raised up to  $1195^\circ$  C., and this temperature was kept for two hours and main sintering was performed. Next, solution treatment and aging were performed under the same conditions as those of the example 2,

whereby a desired sintered magnet was obtained. The composition of the sintered magnet is as shown in Table 1. Regarding the obtained sintered magnet, a density of a sintered compact, a Fe concentration (C1) of a cell phase, a Fe concentration difference (C1-C2) between the cell phase and a cell wall phase, a coercive force, and residual magnetization were measured in the same manner as in the example 1. The measurement results are shown in Table 3.

## Example 9

Alloy powder having the same composition as that of the example 5 was press-formed in a magnetic field, whereby a compression-molded body was fabricated. This compression-molded body was disposed in a chamber of a firing furnace, and the chamber was vacuum-exhausted until its degree of vacuum became  $1.9 \times 10^{-2}$  Pa. In this state, a temperature in the chamber was raised up to 1180° C., and after this temperature was kept for one minute, Ar gas was led into the chamber. The temperature in the chamber set to the Ar atmosphere was raised up to 1198° C., and this temperature was kept for three hours and main sintering was performed. Next, solution treatment and aging were performed under the same conditions as those of the example 5, whereby a desired sintered magnet was obtained. The composition of the sintered magnet is as shown in Table 1. Regarding the obtained sintered magnet, a density of a sintered compact, a Fe concentration (C1) of a cell phase, a Fe concentration difference (C1-C2) between the cell phase and a cell wall phase, a coercive force, and residual magnetization were measured in the same manner as in the example 1. The measurement results are shown in Table 3.

## Example 10

Alloy powder having the same composition as that of the example 1 was press-formed in a magnetic field, whereby a compression-molded body was fabricated. This compression-molded body was disposed in a chamber of a firing furnace, and the chamber was vacuum-exhausted until its degree of vacuum became  $9.5 \times 10^{-3}$  Pa. In this state, a temperature in the chamber was raised up to 1160° C., and after this temperature was kept for fifteen minutes, Ar gas was led into the chamber. The temperature in the chamber set to the Ar atmosphere was raised up to 1195° C., and this temperature was kept for two hours and main sintering was performed. Next, solution treatment and aging were performed under the same conditions as those of the example 1, whereby a desired sintered magnet was obtained. The composition of the sintered magnet is as shown in Table 1. Regarding the obtained sintered magnet, a density of a sintered compact, a Fe concentration (C1) of a cell phase, a Fe concentration difference (C1-C2) between the cell phase and a cell wall phase, a coercive force, and residual magnetization were measured in the same manner as in the example 1. The measurement results are shown in Table 3.

## Example 11

Alloy powder having the same composition as that of the example 5 was press-formed in a magnetic field, whereby a compression-molded body was fabricated. This compression-molded body was disposed in a chamber of a firing furnace, and the chamber was vacuum-exhausted until its degree of vacuum became  $8.5 \times 10^{-3}$  Pa. In this state, a temperature in the chamber was raised up to 1180° C., and after this temperature was kept for ten minutes, Ar gas was

led into the chamber. The temperature in the chamber set to the Ar atmosphere was raised up to 1198° C., and this temperature was kept for three hours and the main sintering was performed. Next, solution treatment and aging were performed under the same conditions as those of the example 5, whereby a desired sintered magnet was obtained. The composition of the sintered magnet is as shown in Table 1. Regarding the obtained sintered magnet, a density of a sintered compact, a Fe concentration (C1) of a cell phase, a Fe concentration difference (C1-C2) between the cell phase and a cell wall phase, a coercive force, and residual magnetization were measured in the same manner as in the example 1. The measurement results are shown in Table 3.

## Example 12

Alloy powder having the same composition as that of the example 5 was press-formed in a magnetic field, whereby a compression-molded body was fabricated. This compression-molded body was disposed in a chamber of a firing furnace, and the chamber was vacuum-exhausted until its degree of vacuum became  $8.5 \times 10^{-3}$  Pa. In this state, a temperature in the chamber was raised up to 1180° C., and after this temperature was kept for ten minutes, the temperature was decreased to room temperature. Next, Ar gas was led into the chamber in the room temperature state and the temperature was raised up to 1198° C., and this temperature was kept for three hours and main sintering was performed. Next, solution treatment and aging were performed under the same conditions as those of the example 5, whereby a desired sintered magnet was obtained. The composition of the sintered magnet is as shown in Table 1. Regarding the obtained sintered magnet, a density of a sintered compact, a Fe concentration (C1) of a cell phase, a Fe concentration difference (C1-C2) between the cell phase and a cell wall phase, a coercive force, and residual magnetization were measured in the same manner as in the example 1. The measurement results are shown in Table 3.

## Comparative Example 1

A sintered magnet having the composition shown in Table 1 was fabricated by employing the same manufacturing method as that of the example 1. Regarding the obtained sintered magnet, a density of a sintered compact, a Fe concentration (C1) of a cell phase, a Fe concentration difference (C1-C2) between the cell phase and a cell wall phase, a coercive force, and residual magnetization were measured in the same manner as in the example 1. They measurement results are shown in Table 3.

## Comparative Example 2

A sintered magnet having the composition shown in Table 1 was fabricated by employing the same manufacturing method as that of the example 5. Regarding the obtained sintered magnet, a density of a sintered compact, a Fe concentration (C1) of a cell phase, a Fe concentration difference (C1-C2) between the cell phase and a cell wall phase, a coercive force, and residual magnetization were measured in the same manner as in the example 1. The measurement results are shown in Table 3.

## Comparative Example 3

Alloy powder having the same composition as that of the example 5 was press-formed in a magnetic field, whereby a

compression-molded body was fabricated. This compression-molded body was disposed in a chamber of a firing furnace, and the chamber was vacuum-exhausted until its degree of vacuum became  $8.5 \times 10^{-3}$  Pa. In this state, a temperature in the chamber was raised up to  $1110^\circ$  C., and after this temperature was kept for one minute, Ar gas was led into the chamber. The temperature in the chamber set to the Ar atmosphere was raised up to  $1198^\circ$  C., and this temperature was kept for three hours and main sintering was performed. Next, solution treatment and aging were performed under the same conditions as those of the example 5, whereby a desired sintered magnet was obtained. The composition of the sintered magnet is as shown in Table 1. Regarding the obtained sintered magnet, a density of a sintered compact, a Fe concentration (C1) of a cell phase, a Fe concentration difference (C1-C2) between the cell phase and a cell wall phase, a coercive force, and residual magnetization were measured in the same manner as in the example 1. The measurement results are shown in Table 3.

#### Comparative Example 4

Alloy powder having the same composition as that of the example 5 was press-formed in a magnetic field, whereby a compression-molded body was fabricated. This compression-molded body was disposed in a chamber of a firing furnace, and the chamber was vacuum-exhausted until its degree of vacuum became  $8.5 \times 10^{-3}$  Pa. In this state, a temperature in the chamber was raised up to  $1135^\circ$  C., and after this temperature was kept for one minute, Ar gas was led into the chamber. The temperature in the chamber set to the Ar atmosphere was raised up to  $1198^\circ$  C., and this temperature was kept for three hours and main sintering was performed. Next, solution treatment and aging were performed under the same conditions as those of the example 5, whereby a desired sintered magnet was obtained. The composition of the sintered magnet is as shown in Table 1. Regarding the obtained sintered magnet, a density of a sintered compact, a Fe concentration (C1) of a cell phase, a Fe concentration difference (C1-C2) between the cell phase and a cell wall phase, a coercive force, and residual magnetization were measured in the same manner as in the example 1. The measurement results are shown in Table 3.

TABLE 1

| Composition of Magnet (at %) |                                                                        |  |  |  |  |
|------------------------------|------------------------------------------------------------------------|--|--|--|--|
| Example 1                    | $Sm_{11.11}Fe_{28.89}(Zr_{0.92}Ti_{0.08})_{2.31}Cu_{6.22}Co_{51.47}$   |  |  |  |  |
| Example 2                    | $(Sm_{0.92}Nd_{0.08})_{10.87}Fe_{29.41}Zr_{1.96}Cu_{5.35}Co_{52.41}$   |  |  |  |  |
| Example 3                    | $Sm_{11.30}Fe_{30.07}Cu_{5.23}Zr_{1.95}(Co_{0.998}Cr_{0.002})_{51.45}$ |  |  |  |  |
| Example 4                    | $Sm_{10.31}Fe_{28.61}Zr_{1.97}Cu_{5.56}Co_{53.55}$                     |  |  |  |  |
| Example 5                    | $Sm_{11.00}Fe_{30.84}Cu_{5.07}Zr_{1.78}Co_{51.31}$                     |  |  |  |  |
| Example 6                    | $Sm_{11.00}Fe_{30.84}Cu_{5.07}Zr_{1.78}Co_{51.31}$                     |  |  |  |  |
| Example 7                    | $Sm_{11.00}Fe_{30.84}Cu_{5.07}Zr_{1.78}Co_{51.31}$                     |  |  |  |  |
| Example 8                    | $(Sm_{0.92}Nd_{0.08})_{10.87}Fe_{29.41}Zr_{1.96}Cu_{5.35}Co_{52.41}$   |  |  |  |  |
| Example 9                    | $Sm_{11.00}Fe_{30.84}Cu_{5.07}Zr_{1.78}Co_{51.31}$                     |  |  |  |  |
| Example 10                   | $Sm_{11.11}Fe_{28.89}(Zr_{0.92}Ti_{0.08})_{2.31}Cu_{6.22}Co_{51.47}$   |  |  |  |  |
| Example 11                   | $Sm_{11.00}Fe_{30.84}Cu_{5.07}Zr_{1.78}Co_{51.31}$                     |  |  |  |  |
| Example 12                   | $Sm_{11.00}Fe_{30.84}Cu_{5.07}Zr_{1.78}Co_{51.31}$                     |  |  |  |  |
| Comparative Example 1        | $Sm_{11.11}Fe_{25.78}(Zr_{0.92}Ti_{0.08})_{2.31}Cu_{6.22}Co_{54.58}$   |  |  |  |  |
| Comparative Example 2        | $Sm_{9.90}Fe_{31.22}Cu_{5.14}Zr_{1.80}Co_{51.94}$                      |  |  |  |  |
| Comparative Example 3        | $Sm_{11.00}Fe_{30.84}Zr_{1.78}Cu_{5.07}Co_{51.31}$                     |  |  |  |  |
| Comparative Example 4        | $Sm_{11.00}Fe_{30.84}Zr_{1.78}Cu_{5.07}Co_{51.31}$                     |  |  |  |  |

TABLE 2

| 5  | Pre-Process Step<br>(vacuum process step) |                                                                  |                                                     | Main Sintering Step           |                                                  |                      |
|----|-------------------------------------------|------------------------------------------------------------------|-----------------------------------------------------|-------------------------------|--------------------------------------------------|----------------------|
|    | Process                                   | Temperature T<br>(Atmosphere<br>Change<br>Temperature)<br>[° C.] | Degree<br>of<br>Vacuum<br>[ $\times 10^{-3}$<br>Pa] | Retention<br>Time<br>[minute] | Main<br>Sintering<br>Temperature<br>Ts<br>[° C.] | Ts –<br>50<br>[° C.] |
|    |                                           |                                                                  |                                                     |                               |                                                  |                      |
| 10 | Example 1                                 | 1160                                                             | 9.0                                                 | 5                             | 1195                                             | 1145                 |
| 15 | Example 2                                 | 1160                                                             | 9.0                                                 | 5                             | 1195                                             | 1145                 |
| 20 | Example 3                                 | 1185                                                             | 9.0                                                 | 1                             | 1195                                             | 1145                 |
| 25 | Example 4                                 | 1180                                                             | 8.0                                                 | 20                            | 1205                                             | 1155                 |
| 30 | Example 5                                 | 1180                                                             | 8.5                                                 | 1                             | 1198                                             | 1148                 |
| 35 | Example 6                                 | 1190                                                             | 8.5                                                 | 1                             | 1198                                             | 1148                 |
| 40 | Example 7                                 | 1155                                                             | 8.5                                                 | 1                             | 1198                                             | 1148                 |
| 45 | Example 8                                 | 1160                                                             | 2.8                                                 | 5                             | 1195                                             | 1145                 |
| 50 | Example 9                                 | 1180                                                             | 1.9                                                 | 1                             | 1198                                             | 1148                 |
| 55 | Example 10                                | 1160                                                             | 9.5                                                 | 15                            | 1195                                             | 1145                 |
| 60 | Example 11                                | 1180                                                             | 8.5                                                 | 10                            | 1198                                             | 1148                 |
| 65 | Example 12                                | 1180                                                             | 8.5                                                 | 10                            | 1198                                             | 1148                 |
| 70 | Comparative Example 1                     | 1160                                                             | 9.0                                                 | 5                             | 1195                                             | 1145                 |
| 75 | Comparative Example 2                     | 1180                                                             | 8.5                                                 | 1                             | 1198                                             | 1148                 |
| 80 | Comparative Example 3                     | 1110                                                             | 8.5                                                 | 1                             | 1198                                             | 1148                 |
| 85 | Comparative Example 4                     | 1135                                                             | 8.5                                                 | 1                             | 1198                                             | 1148                 |

TABLE 3

| 35                    | Density of Sintered Compact<br>[ $\times 10^3$ kg/m <sup>3</sup> ] | Fe Concentration of Cell Phase<br>[at %] | Fe Concentration Between Cell Phase and Cell Wall Phase<br>[at %] | Coercive Force<br>[kA/m] | Residual Magnetization<br>[T] |
|-----------------------|--------------------------------------------------------------------|------------------------------------------|-------------------------------------------------------------------|--------------------------|-------------------------------|
|                       |                                                                    |                                          |                                                                   |                          |                               |
| Example 1             | 8.27                                                               | 29.3                                     | 16.5                                                              | 1180                     | 1.18                          |
| Example 2             | 8.28                                                               | 29.8                                     | 18.7                                                              | 1090                     | 1.19                          |
| Example 3             | 8.31                                                               | 30.1                                     | 14.4                                                              | 1075                     | 1.20                          |
| Example 4             | 8.28                                                               | 28.8                                     | 12.5                                                              | 835                      | 1.19                          |
| Example 5             | 8.25                                                               | 31.2                                     | 20.8                                                              | 1150                     | 1.18                          |
| Example 6             | 8.27                                                               | 31.8                                     | 21.5                                                              | 1175                     | 1.19                          |
| Example 7             | 8.22                                                               | 30.9                                     | 16.4                                                              | 1100                     | 1.16                          |
| Example 8             | 8.24                                                               | 29.5                                     | 13.4                                                              | 965                      | 1.16                          |
| Example 9             | 8.22                                                               | 30.7                                     | 12.2                                                              | 870                      | 1.15                          |
| Example 10            | 8.30                                                               | 30.0                                     | 19.7                                                              | 1225                     | 1.20                          |
| Example 11            | 8.30                                                               | 32.1                                     | 22.2                                                              | 1190                     | 1.21                          |
| Example 12            | 8.29                                                               | 32.3                                     | 23.0                                                              | 1205                     | 1.21                          |
| Comparative Example 1 | 8.30                                                               | 26.1                                     | 14.2                                                              | 1710                     | 1.10                          |
| Comparative Example 2 | 7.65                                                               | 31.3                                     | 7.8                                                               | 95                       | 1.07                          |
| Comparative Example 3 | 7.46                                                               | 30.7                                     | 4.1                                                               | 120                      | 1.04                          |
| Comparative Example 4 | 7.89                                                               | 30.8                                     | 7.9                                                               | 370                      | 1.09                          |

As is apparent from Table 3, it is seen that the sintered magnets of the examples 1 to 12 all have a high density and have a large Fe concentration difference between the cell phase and the cell wall phase, and as a result, they all have high magnetization and a high coercive force. Having a low Fe concentration, the sintered magnet of the comparative example 1 has low magnetization even though the density is high. Having a low Sm concentration, the sintered magnet of the comparative example 2 is low both in the magnetization and the coercive force. The sintered magnets of the comparative examples 3, 4 are low in the density of the sintered compact even though their Fe concentration is high, and are

## 21

low both in the magnetization and the coercive force due to the small Fe concentration difference between the cell phase and the cell wall phase.

While certain embodiments have been described, these embodiments have been presented by way of example only, and are not intended to limit the scope of the inventions. Indeed, the novel embodiments described herein may be embodied in a variety of other forms; furthermore, various omissions, substitutions and changes in the form of the embodiments described herein may be made without departing from the spirit of the inventions. The accompanying claims and their equivalents are intended to cover such forms or modifications as would fall within the scope and spirit of the inventions.

What is claimed is:

1. A permanent magnet comprising a sintered compact, the sintered compact comprising:  
a composition expressed by the following composition formula:



wherein, R is at least one element selected from the group consisting of rare-earth elements, and 50 at % or more of the element R is Sm,

M is at least one element selected from the group consisting of Zr, Ti, and Hf,

p is a number satisfying  $10 < p < 13.5$  at %,

q is a number satisfying  $30 < q < 40$  at %,

r is a number satisfying  $1.78 < r < 7.2$  at %, and

s is a number satisfying  $3.5 < s < 13.5$  at %; and  
a metallic structure including a cell phase having a

$Th_2Zn_{17}$  crystal phase, and a cell wall phase surrounding the cell phase,

wherein a Fe concentration (C1) in the cell phase is in a range from 30.1 at % to 32.3 at %, and a difference (C1-C2) between the Fe concentration (C1) in the cell phase and a Fe concentration (C2) in the cell wall phase is in a range from 12.2 at % to 23.0 at %,

wherein the sintered compact has a density of  $8.22 \times 10^3$  kg/m<sup>3</sup> or more and  $8.31 \times 10^3$  kg/m<sup>3</sup> or less, and

wherein a coercive force of the permanent magnet is 870 kA/m or more.

2. The permanent magnet of claim 1, wherein 50 at % or more of the element M is Zr.

## 22

3. The permanent magnet of claim 1, wherein r is a number satisfying  $1.95 \leq r \leq 7.2$  at %.

4. A motor comprising the permanent magnet of claim 1.

5. A power generator comprising the permanent magnet of claim 1.

6. The motor of claim 4, further comprising:

a stator; and

a rotor, arranged in the stator, comprising the permanent magnet.

7. The power generator of claim 5, further comprising:  
a stator comprising the permanent magnet; and  
a rotor arranged in the stator.

8. A vehicle comprising the motor of claim 4.

9. A vehicle comprising the power generator of claim 5.

10. A permanent magnet comprising a sintered compact, the sintered compact comprising:

a composition expressed by the following composition formula:



20 wherein, R is at least one element selected from the group consisting of rare-earth elements, and 50 at % or more of the element R is Sm,

M is at least one element selected from the group consisting of Zr, Ti, and Hf,

A is at least one element selected from the group consisting of Ni, V, Cr, Mn, Al, Ga, Nb, Ta, and W,

p is a number satisfying  $10 \leq p \leq 13.5$  at %,

q is a number satisfying  $30 \leq q \leq 40$  at %,

r is a number satisfying  $1.78 \leq r \leq 7.2$  at %,

s is a number satisfying  $3.5 \leq s \leq 13.5$  at %, and

$\alpha$  is a number satisfying  $\alpha \leq 20$  at %; and

a metallic structure including a cell phase having a  $Th_2Zn_{17}$  crystal phase, and a cell wall phase surrounding the cell phase,

wherein a Fe concentration (C1) in the cell phase is in a range from 30.1 at % to 32.3 at %, and a difference (C1-C2) between the Fe concentration (C1) in the cell phase and a Fe concentration (C2) in the cell wall phase is in a range from 12.2 at % to 23.0 at %,

wherein the sintered compact has a density of  $8.22 \times 10^3$  kg/m<sup>3</sup> or more and  $8.31 \times 10^3$  kg/m<sup>3</sup> or less, and

wherein a coercive force of the permanent magnet is 870 kA/m or more.

\* \* \* \* \*